

May 8, 1923.

1,454,200

J. C. WELLS ET AL

ANTAEUS GLASS

Filed May 13, 1922



FIG. I



FIG. II



FIG. III



FIG. IV



FIG. V



FIG. VI



FIG. VII



FIG. VIII

INVENTOR  
J. C. WELLS  
E. D. TILLYER  
BY

H. H. Styll & H. Parsons  
ATTORNEYS

Patented May 8, 1923.

1,454,200

# UNITED STATES PATENT OFFICE.

JOEL C. WELLS AND EDGAR D. TILLYER, OF SOUTHBRIIDGE, MASSACHUSETTS; SAID TILLYER ASSIGNOR TO SAID WELLS.

## ANTÆUS GLASS.

Application filed May 13, 1922. Serial No. 560,614.

*To all whom it may concern:*

Be it known that we, JOEL C. WELLS and EDGAR D. TILLYER, citizens of the United States, residing at Southbridge, in the 5 county of Worcester and State of Massachusetts, have invented certain new and useful Improvements in New Antæus Glass, of which the following is a specification.

This invention relates to a new and useful process in the forming of ophthalmic lenses and more particularly to a process whereby lenses of this character will be produced which will withstand comparatively heavy blows or pressure upon the convex 15 surface of the lens so that they will be especially valuable for use in various types of goggles and the like.

The main object of our invention is the process of forming a lens particularly 20 adapted for use in goggles and the like where it is sometimes necessary to have the convex surface of the lens withstand a comparatively heavy blow with the assurance of the fact that the lens will not be shattered 25 or broken over the contact of the blow and thus protect the eyes of the wearer.

A further object of our invention is the process of forming a hardened lens which consists in heating a lens blank to produce 30 a convex surface and then suddenly cooling this convex surface causing the same to contract in the cooling of the concave surface slowly which will tend to exert a pull on the hardened convex surface producing a compression in the convex surface and a tension 35 in the concave surface.

A further object of the invention is the provision of a lens of the above character which can be produced at a comparatively 40 low cost and which at the same time will provide an effective protection for the eyes of the wearer.

With the above and other objects in view the invention consists in the novel features of 45 construction, the combination and arrangement of parts hereinafter more fully set forth, pointed out in the claims and shown in the accompanying drawings, in which—

Figure I is a front elevation of a pair of 50 goggles including our improved lens.

Figure II is a side elevation of a non-finished lens blank.

Figure III is a side elevation of a finished lens blank.

Figure IV is a transverse section of a

heating furnace for producing the concave on the lens.

Figure V is a vertical section illustrating the lens upon the supporting ring prior to heating. 60

Figure VI is a transverse section showing the lens in a reformed condition.

Figure VII is a longitudinal section thru a cooling device showing the lens in position for cooling the convex surface, and 65

Figure VIII is a longitudinal sectional view of a finished lens constructed in accordance with our improved process.

Referring to the drawings which we have used for illustrating the use of our improved 70 lens and the manner of carrying out the process, the numeral 1 indicates the lens frames of a pair of goggles in which the lenses 2 are mounted. The goggles are provided with the usual temples 3 for supporting the same upon the face of the wearer, the lenses illustrated herein being of our improved type. 75

The process of forming our improved lens consists in taking a rough lens blank 4 which is shown in Figure II for grinding and polishing the opposed surfaces of the lenses until they are ground down to the proper thickness as shown in Figure III. It is preferred to have the surfaces of the lens 85 polished prior to hardening as will be set forth hereafter as the hardening of the lens will not destroy polished surfaces. 80

In Figure III the lens is shown with two polished surfaces 5 and 6 and after a lens has been polished to the required condition it is placed upon a supporting ring 7 having an inwardly inclined bevel portion 8 as illustrated in Figure V. 90

The ring 7 is preferably arranged within 95 a heating furnace 9 and the lens 4 arranged within the furnace and mounted upon the upper edge of the ring. The furnace 9 is heated to the required temperature which will soften the lens and cause the lower surface thereof to drop downwardly as illustrated in Figure VI, the face of the lens adjacent the edge resting upon the inclined surface 8 to thus produce a true arc on the convex surface of the lens. In order to regulate the required amount of temperature necessary to cause the lens to drop as shown in Figure VI a thermometer 10 is arranged within the furnace with the upper end projecting thru the roof of the furnace so that 100 105 110

the temperature may be readily regulated by the operator.

- 5 After the lens has been heated and formed to the proper shape as illustrated in Figure VI it is quickly transferred to a cooling device which includes the supporting plate 11 having a chamber 12 arranged beneath the plate in the form of a concave pocket and communicating with the chamber is an inlet 10 tube 13 which communicates with the interior of the chamber 12 to provide a suitable air pressure which is distributed over the convex surface 6 of the lens by means of a plurality of perforations 14 formed in the 15 plate 11 whereby the convex surface of the lens will be quickly cooled which will cause the same to contract, set and harden while the upper or concave surface of the lens is in a softened state.
- 20 Attention is called to the fact that when the soft surface on the concave side of the lens begins to cool it will slowly tend to produce a pulling on the hardened convex surface of the lens producing a compression in 25 the convex surface 6 of the lens and a tension in the concave surface 5 of the lens.

In Figure VIII the direction of the arrows on the convex surface of the lens illustrates the direction in which the contraction takes place while the arrows on the concave surface indicates the expansion of the softened selfside of the lens prior to cooling.

30 From the above it will be apparent that after a lens has been put thru the above process, the convex surface of the lens will be in a sufficiently heated condition to withstand comparatively severe blows on the 35 surface of the lens without the lens being shattered or broken over the contact of the blow.

In the art of manufacturing glass it is a well known fact that glass under compression is much stronger than glass under tension and it is, therefore, one of the principal objects of our process to produce compression upon the convex surface of the lens with a tension in the concave surface as it is

the convex surface of the lens which must withstand any blows.

50 It will also be apparent that our improved process is comparatively inexpensive to carry out and at the same time will produce a lens which will be extremely effective for the use to which it is to be applied.

55 We claim:

1. The process of producing protection lenses consisting in heating the lens uniformly and subsequently cooling one face of the lens while the other is in a plastic 60 condition.

2. The process of producing a tempered lens consisting in uniformly heating the lens blank, suddenly cooling one surface thereof, and allowing the opposite surface to cool 65 naturally.

3. The process of producing a tempered lens consisting in finishing the surfaces of a glass blank, subjecting the parts to heat which will drop the finished blank to desired 70 curve and suddenly chilling one face of the blank to produce a surface tension thereof.

4. As an article of manufacture a lens blank having opposite inherent stresses on the respective faces thereof.

75 5. The process of producing a curved protection lens consisting in surfacing the faces of the lens in flat form, subjecting the blanks after surfacing to sufficient heat to drop the lens to desired curve without impairment of the polished surfaces thereof, and suddenly chilling one face of the blank to produce a surface tension in the finished blank, increasing the resisting properties thereof.

80 6. The process of producing a shock resisting ophthalmic lens consisting in heating the lens to a plastic condition and causing one face of the lens to harden and set in advance of the other whereby the contraction of the later cooling surface will produce a compression as respects the first cooled surface, causing a surface tension effect therein.

JOEL C. WELLS.  
EDGAR D. TILLYER.